

# United States Patent Office

2,757,133

Patented July 31, 1956

1

2,757,133

## ELECTRODEPOSITION OF NICKEL

Wilbur J. Shenk, Jr., Shaker Heights, Ohio, assignor to The Harshaw Chemical Company, Elyria, Ohio, a corporation of Ohio

No Drawing. Application June 10, 1952,  
Serial No. 292,725

17 Claims. (Cl. 204—49)

This invention relates to electrodeposition of nickel, and more specifically to the use of certain addition agents which effectively enhance brightness and improve ductility.

It is recognized that prior to the present invention a great variety of organic addition agents have been used or proposed for use for the production of bright or semi-bright nickel deposits. Some of these have proved to be of commercial value, while others have failed because of their sensitivity to impurities or failure to continue producing good deposits over sufficiently long periods of time. Some of the proposed addition agents have not been commercialized merely because other addition agents were found to be somewhat superior. Such considerations as the rate of consumption in the plating solution, the difficulty of analyzing the solution or otherwise determining the concentration of brightener, and the build-up of the concentration of degradation products are important in the choice of brightening addition agents.

The present invention has to do with the use, either as the sole brightening addition agent or as a cooperating addition agent for use with other brighteners, of a class of compounds, one representative of which is a compound known as dibenzenesulfonamide or dibenzenesulfonyl amine and having the formula,



Other examples of the class are:

TABLE I

- (1) Trichlorodibenzenesulfonamides-  
 $\text{Cl}_2\text{C}_6\text{H}_3\text{SO}_2\text{NHSO}_2\text{C}_6\text{H}_4\text{Cl}$
- (2) Tetrachlorodibenzenesulfonamides-  
 $\text{Cl}_2\text{C}_6\text{H}_3\text{SO}_2\text{NHSO}_2\text{C}_6\text{H}_3\text{Cl}_2$
- (3) Di- $\beta$ -naphthalenesulfonamide-  
 $\text{C}_{10}\text{H}_7\text{SO}_2\text{NHSO}_2\text{C}_{10}\text{H}_7$
- (4) 2,2',4,4',6,6'-Hexachlorodibenzenesulfonamide-  
 $\text{Cl}_3\text{C}_6\text{H}_2\text{SO}_2\text{NHSO}_2\text{C}_6\text{H}_2\text{Cl}_3$
- (5) Pentachlorodibenzenesulfonamides-  
 $\text{Cl}_3\text{C}_6\text{H}_2\text{SO}_2\text{NHSO}_2\text{C}_6\text{H}_3\text{Cl}_2$
- (6) Methylchlorodibenzenesulfonamides-  
 $\text{Cl}_2\text{C}_6\text{H}_3\text{SO}_2\text{NHSO}_2\text{C}_6\text{H}_4\text{CH}_3$
- (7) 2,4,6-Trichlorodibenzenesulfonamide-  
 $\text{Cl}_3\text{C}_6\text{H}_2\text{SO}_2\text{NHSO}_2\text{C}_6\text{H}_5$
- (8) 2,5-Dichloro-3'-sulfamylbenzenesulfonamide-  
 $\text{Cl}_2\text{C}_6\text{H}_3\text{SO}_2\text{NHSO}_2\text{C}_6\text{H}_4\text{SO}_2\text{NH}_2$
- (9) Disulfonilamide- $\text{NH}_2\text{C}_6\text{H}_4\text{SO}_2\text{NHSO}_2\text{C}_6\text{H}_4\text{NH}_2$
- (10) N-phenylsulfonyl- $\beta$ -naphthalenesulfonamide-  
 $\text{C}_6\text{H}_5\text{SO}_2\text{NHSO}_2\text{C}_10\text{H}_7$

2

- (11) Di-p-toluenesulfonamide-  
 $\text{CH}_3\text{C}_6\text{H}_4\text{SO}_2\text{NHSO}_2\text{C}_6\text{H}_4\text{CH}_3$
- 5 (12) 4-Methyldibenzenesulfonamide-  
 $\text{C}_6\text{H}_5\text{SO}_2\text{NHSO}_2\text{C}_6\text{H}_4\text{CH}_3$
- (13) N,N'-bis(phenylsulfonyl)-m-sulfamylbenzamide-  
 $\text{C}_6\text{H}_5\text{SO}_2\text{NHSO}_2\text{C}_6\text{H}_4\text{CONHSO}_2\text{C}_6\text{H}_5$
- 10 (14) Dicumenesulfonamide-  
 $(\text{CH}_3)_2\text{CHC}_6\text{H}_4\text{SO}_2\text{NHSO}_2\text{C}_6\text{H}_4\text{CH}(\text{CH}_3)_2$
- (15) 4-Ethyldibenzenesulfonamide-  
 $\text{C}_6\text{H}_5\text{SO}_2\text{NHSO}_2\text{C}_6\text{H}_4\text{C}_2\text{H}_5$
- (16) 4,4'-Dicarboxyldibenzenesulfonamide-  
 $\text{COOHC}_6\text{H}_4\text{SO}_2\text{NHSO}_2\text{C}_6\text{H}_4\text{COOH}$
- 20 (17) 2,2',4,4'-Tetramethyldibenzenesulfonamide-  
 $(\text{CH}_3)_2\text{C}_6\text{H}_3\text{SO}_2\text{NHSO}_2\text{C}_6\text{H}_3(\text{CH}_3)_2$
- (18) Dichlorodibenzenesulfonamides-  
 $\text{Cl}_2\text{C}_6\text{H}_3\text{SO}_2\text{NHSO}_2\text{C}_6\text{H}_5$
- 25 (19) 4-Fluorodibenzenesulfonamides-  
 $\text{FC}_6\text{H}_4\text{SO}_2\text{NHSO}_2\text{C}_6\text{H}_5$
- (20) 4-Carboxyldibenzenesulfonamide-  
 $\text{C}_6\text{H}_5\text{SO}_2\text{NHSO}_2\text{C}_6\text{H}_4\text{COOH}$
- 30 (21) N,N'-bis-(phenylsulfonyl)-1,3-benzenedisulfonamide-  
 $\text{C}_6\text{H}_5\text{SO}_2\text{NHSO}_2\text{C}_6\text{H}_4\text{SO}_2\text{NHSO}_2\text{C}_6\text{H}_5$
- (22) N,N'-bis(dichlorophenylsulfonyl)-1,3-benzenedisulfonamides-  
 $\text{Cl}_2\text{C}_6\text{H}_3\text{SO}_2\text{NHSO}_2\text{C}_6\text{H}_4\text{SO}_2\text{NHSO}_2\text{C}_6\text{H}_3\text{Cl}_2$
- 35 (23) N,N'-bis(phenylsulfonyl)-4,4'-diphenyldisulfonamide-  
 $\text{C}_6\text{H}_5\text{SO}_2\text{NHSO}_2\text{C}_6\text{H}_4\text{C}_6\text{H}_4\text{SO}_2\text{NHSO}_2\text{C}_6\text{H}_5$
- (24) p,p'-Oxy-bis(dibenzenesulfonamide)-  
 $\text{C}_6\text{H}_5\text{SO}_2\text{NHSO}_2\text{C}_6\text{H}_4\text{OC}_6\text{H}_4\text{SO}_2\text{NHSO}_2\text{C}_6\text{H}_5$
- (25) p,p'-Methylene-bis(dibenzenesulfonamide)-  
40  $\text{C}_6\text{H}_5\text{SO}_2\text{NHSO}_2\text{C}_6\text{H}_4\text{CH}_2\text{C}_6\text{H}_4\text{SO}_2\text{NHSO}_2\text{C}_6\text{H}_5$
- (26) N,N'-bis(2,4,6-trichlorophenylsulfonyl)-1,3-benzenedisulfonamide-  
45  $\text{Cl}_3\text{C}_6\text{H}_2\text{SO}_2\text{NHSO}_2\text{C}_6\text{H}_4\text{SO}_2\text{NHSO}_2\text{C}_6\text{H}_2\text{Cl}_3$
- (27) N,N'-bis-(p-tolylsulfonyl)-4,4'-diphenyldisulfonamide-  
50  $\text{CH}_3\text{C}_6\text{H}_4\text{SO}_2\text{NHSO}_2\text{C}_6\text{H}_4\text{C}_6\text{H}_4\text{SO}_2\text{NHSO}_2\text{C}_6\text{H}_4\text{CH}_3$
- (28) N-ethylsulfonylbenzenesulfonamide-  
55  $\text{C}_6\text{H}_5\text{SO}_2\text{NHSO}_2\text{CH}_2\text{CH}_3$
- (29) N-vinylsulfonylbenzenesulfonamide-  
 $\text{C}_6\text{H}_5\text{SO}_2\text{NHSO}_2\text{CH}=\text{CH}_2$
- (30) N-(n-butylsulfonyl)benzenesulfonamide-  
60  $\text{C}_6\text{H}_5\text{SO}_2\text{NHSO}_2\text{C}_4\text{H}_9$
- (31) N-(n-laurylsulfonyl)-benzenesulfonamide-  
 $\text{C}_6\text{H}_5\text{SO}_2\text{NHSO}_2\text{C}_{12}\text{H}_{25}$
- (32) Di- $\alpha$ -toluenesulfonamide-  
 $\text{C}_6\text{H}_5\text{CH}_2\text{SO}_2\text{NHSO}_2\text{CH}_2\text{C}_6\text{H}_5$
- 65 (33) N-benzylsulfonylbenzenesulfonamide-  
 $\text{C}_6\text{H}_5\text{SO}_2\text{NHSO}_2\text{CH}_2\text{C}_6\text{H}_5$
- (34) N-ethylsulfonyldichlorobenzenesulfonamides-  
 $\text{Cl}_2\text{C}_6\text{H}_3\text{SO}_2\text{NHSO}_2\text{C}_2\text{H}_5$
- 70 (35) N-methylsulfonylbenzenesulfonamide-  
 $\text{C}_6\text{H}_5\text{SO}_2\text{NHSO}_2\text{CH}_2\text{C}(\text{CH}_3)=\text{CH}_2$

## 3

(36) N-methylsulfonylbenzenesulfonamide-

(37) Dimethanesulfonamide- $\text{CH}_3\text{SO}_2\text{NHSO}_2\text{CH}_3$  (Inoperative)(38) Didodecanesulfonamide -  $\text{C}_{12}\text{H}_{25}\text{SO}_2\text{NHSO}_2\text{C}_{12}\text{H}_{25}$  (Inoperative)

(39) N,N'-bis(phenylsulfonyl)-1,5-naphthalenedisulfonamide

(40) N,N'-bis(phenylsulfonyl)3,3'-benzophenonedisulfonamide- $\text{C}_6\text{H}_5\text{SO}_2\text{NHSO}_2\text{C}_6\text{H}_4\text{COC}_6\text{H}_4\text{SO}_2\text{NHSO}_2\text{C}_6\text{H}_5$ 

The indicated class of compounds which may be called disulfonamides or disulfonyl amines are effective both alone and in cooperation with a wide variety of auxiliary brighteners in the production respectively of semi-bright and bright deposits over long periods of operation. These compounds are very strongly acidic as compared to compounds of the type  $\text{RSO}_2\text{NH}_2$ . For example,



has a pH of 1.3 in tenth normal solution whereas



is only about as acidic as phenol. Again, they are very soluble in water. For example,  $\text{PhSO}_2\text{NHSO}_2\text{Ph}$  is soluble in water at 20°C. to the extent of about 50 grams per liter, while  $\text{PhSO}_2\text{NH}_2$  is soluble under the same conditions only to the extent of about 3 grams per liter. This solubility difference increases in importance as one considers nuclear substitution products of benzenesulfonamide which have less solubility. Thus 2,5-dichlorobenzenesulfonamide,  $\text{Cl}_2\text{C}_6\text{H}_3\text{SO}_2\text{NH}_2$ , appears to have promise as a scratch-filling carrier in certain bright baths, but its low solubility, 0.5 g./l. in Watts bath solution, severely limits its usefulness. On the other hand, 2,5-dichlorodibenzenesulfonamide,  $\text{Cl}_2\text{C}_6\text{H}_3\text{SO}_2\text{NHSO}_2\text{C}_6\text{H}_3$ , has a solubility of approximately 30 g./l. in the Watts bath, thus permitting its use over a wide range of concentrations, and it has been found to be an excellent scratch-filling carrier.

It has been established that 2,5-dichlorodibenzenesulfonamide is slowly converted principally to dibenzenesulfonamide by hydrogenolysis during the plating operation, and it appears that the superior leveling properties of the bath containing this compound are in some way related to this reaction which is presumably taking place catalytically on the freshly deposited nickel surface.

If one tries to increase the degree of halogenation to say 2,2',5,5'-tetrachlorodibenzenesulfonamide low solubility (in this case about 1 g./l.) again becomes a limiting factor but this can be overcome by using a compound containing two disulfonamide groups. Thus, N,N'-bis(2,5-dichlorophenylsulfonyl)-1,3-benzenedisulfonamide,  $\text{Cl}_2\text{C}_6\text{H}_3\text{SO}_2\text{NHSO}_2\text{C}_6\text{H}_4\text{SO}_2\text{NHSO}_2\text{C}_6\text{H}_3\text{Cl}_2$ , is soluble to an extent of more than 100 g./l. and excellent scratch-filling deposits have been obtained with it. The compound  $\text{Cl}_2\text{C}_6\text{H}_3\text{SO}_2\text{NHSO}_2\text{C}_6\text{H}_5$  has a water solubility of about 3%, the compound  $\text{Cl}_2\text{C}_6\text{H}_3\text{SO}_2\text{NHSO}_2\text{C}_6\text{H}_3\text{Cl}_2$  about 0.1% and the compound  $\text{Cl}_2\text{C}_6\text{H}_3\text{SO}_2\text{NH}_2$  less than 0.1%.

The following formulae indicate desirable classes of compounds for use in accordance with the invention:

TABLE II



## 4

*n* and *n'* each indicating an integer from 0 to 3 and the sum of *n* plus *n'* not exceeding 3.



*n* and *n'* each indicating an integer from 0 to 3 and the sum of *n* plus *n'* not exceeding 6.



*n* and *n'* each indicating an integer from 0 to 3 and the sum of *n* plus *n'* not exceeding 6.



*n* and *n'* each indicating an integer from 0 to 3, and the sum of *n* plus *n'* not exceeding 6.



*n* and *n'* each indicating an integer from 0 to 1.

(7)  $\text{C}_6\text{H}_5\text{SO}_2\text{NHSO}_2\text{C}_6\text{H}_4\text{COC}_6\text{H}_4\text{SO}_2\text{NHSO}_2\text{C}_6\text{H}_5$ 

These compounds indicated in Tables I and II are examples of the class of disulfonamides which produce semi-bright to bright deposits when used in the acid nickel plating solution as the sole brightener, for example in a solution of the Watts type, which might, for example, contain 240 grams per liter of nickel sulfate hexahydrate, 40 grams per liter of nickel chloride hexahydrate, and 40 grams per liter of boric acid, remainder water. It is to be understood that such a nickel plating bath would normally contain an anti-pit agent of the wetting-agent type, such for example as sodium lauryl sulfate or other aliphatic sulfate having 8 to 18 carbon atoms or mixtures thereof, and that the same might be present within the limits of solubility but preferably about 0.1 to 0.5 grams per liter. The anti-pit agent is not always necessary, since the bath sometimes produces pit-free deposits without it, and sometimes the degree of pitting is such as can be tolerated even though some pits are present.

As above indicated, the novel class of compounds can be effectively used in combination with a wide variety of other brighteners, with the result that there is produced bright, ductile deposits having good throwing power and capable of being operated trouble-free for long periods of time. Examples of such cooperating brighteners are as follows:

TABLE III

(1) Ethylene cyanohydrin

(2) Vinyl pyridine

(3) Triaminotriphenylmethane

(4) N-Methylquinuclidinium methyl sulfate

(5) Allyl alcohol

(6) Succinonitrile

(7) Cyclohexanone oxime

(8) Butyraldoxime

(9) Benzaldehyde

(10) N-Methylisoquinolinium methyl sulfate

(11) N-methylpyridinium methyl sulfate

(12) Pyruvic aldehyde

(13) Barbituric acid

The disulfonamides contemplated by the invention for use in nickel plating solutions are of the character indicated by the foregoing examples, that is, they are compounds of the type:



where (1) R and R' both may be aromatic radicals, or (2) R may be an aromatic radical while R' is an aliphatic radical, or (3) both R and R' may be aliphatic or aryl substituted aliphatic radicals. The aromatic radicals should in all instances be limited to not more than 10 nuclear carbons and may carry one or a plurality of substituents of the class chlorine, bromine, fluorine, methyl, ethyl, carboxyl, sulfamyl, R'SO<sub>2</sub>NHSO<sub>2</sub>R,



OR'SO<sub>2</sub>NHSO<sub>2</sub>R and SO<sub>2</sub>NHSO<sub>2</sub>R. The aliphatic radicals, when both R and R' are aliphatic, must contain at least 2 but should not contain more than 18 carbon atoms, must have at least one unsaturated carbon to carbon bond, which, however, may be in an aryl substituent, and may carry one or a plurality of substituents of the class consisting of chlorine, bromine, fluorine, methyl, ethyl, carboxyl, R'SO<sub>2</sub>NHSO<sub>2</sub>R, CH<sub>2</sub>R'SO<sub>2</sub>NHSO<sub>2</sub>R, OR'SO<sub>2</sub>NHSO<sub>2</sub>R and SO<sub>2</sub>NHSO<sub>2</sub>R. When R is aromatic and R' is aliphatic, R should be limited to not more than 10 carbon atoms and R' may be saturated or unsaturated and may contain from 1 to 18 carbon atoms. Either R or R' in that case may be substituted by chlorine, bromine, fluorine, carboxyl or sulfamyl, aryl having not more than 6 carbon atoms, R'SO<sub>2</sub>NHSO<sub>2</sub>R, CH<sub>2</sub>R'SO<sub>2</sub>NHSO<sub>2</sub>R, OR'SO<sub>2</sub>NHSO<sub>2</sub>R or SO<sub>2</sub>NHSO<sub>2</sub>R. In other words, R is an organic radical of the class consisting of aromatic radicals having not more than ten nuclear carbon atoms and aliphatic radicals having at least one unsaturated carbon to carbon bond, and R' is selected from the class consisting of aromatic radicals having not more than ten nuclear carbon atoms, aliphatic radicals having from 1 to 18 carbon atoms, aryl substituted aliphatic radicals having from 7 to 11 carbon atoms, and radicals of the formula R—SO<sub>2</sub>NHSO<sub>2</sub>R.

In general, the concentration of the disulfonamide should be from 0.2 to 6 grams per liter, preferably from 0.5 to 6.0 grams per liter when used as the sole brightening addition agent in a Watts type bath to produce a semi-bright deposit. When used in conjunction with aryl sulfonic acids, sulfonates, sulfonamides or sulfimides, which are themselves effective to produce semi-bright deposits and, in cooperation with auxiliary brighteners such as those listed above, to produce fully bright deposits, the concentration may vary from a very small amount, for example 0.1 gram per liter up to 6 grams per liter, and may be expected to perform its function to a degree in proportion to its concentration. The auxiliary brightening addition agents such as ethylene cyanohydrin and others listed above may be present in various concentrations, ordinarily quite small, and up to such concentration as tends to embrittle the deposit excessively. Suitable concentrations of various auxiliary brightening addition agents are as indicated in the specific examples herein-after set forth.

The constituents of the bath according to the preferred practice of the invention are: (1) water; (2) nickel sulfate, nickel chloride, or nickel sulfate with nickel chloride; (3) a disulfonamide of the class above indicated or a plurality thereof; (4) a wetting agent such as sodium lauryl sulfate or a mixture of aliphatic sulfates having from 8 to 18 carbon atoms, the wetting agent being optional; and (5) an auxiliary brightening addition agent such as those listed above, the auxiliary brightening addition agent also being optional. An additional ingredient of the solution which is desirable is a buffering agent such as boric acid, formic acid, or the like.

It will be noted that in respect to major constituents, the solutions are similar to the well-known "all sulfate," "all chloride," and "sulfate-chloride" or Watts type acid 70 nickel plating solutions. It will be noted also that the auxiliary brighteners such as ethylene cyanohydrin and others listed therewith above are, for the most part, conventional auxiliary brighteners for use with aromatic sulfonic acids and sulfonamides. The essence of the

present invention is in the use of dibenzenesulfonamide and/or other compounds listed above, it having been discovered that this class of compounds, either as the sole brightening addition agent or as a cooperating brightening addition agent, imparts to the bath unexpected properties of bright throwing power, ductility and smoothness. A further important feature of the invention is the use of dibenzenesulfonamide and the other members of its group as above indicated, in solutions which already 10 contain aromatic sulfonic acids, sulfonates or sulfonamides as a partial substitute for those compounds for the purpose of imparting the unexpected properties indicated above. In other words, the dibenzenesulfonamide type of addition agent imparts superior bright throwing power, ductility and smoothness to bright plating solutions of the type wherein principal reliance is placed on a combination of a mononuclear aromatic sulfonyl compound and an auxiliary brightening agent. In conventional solutions, the aromatic sulfonate, for example naphthalene sulfonate, is often referred to as a carrier, while an auxiliary brightener such as triaminotriphenylmethane is referred to as the brightener. In this terminology the disulfonamide is useful either as carrier or as a partial substitute for the usual type of carrier to impart enhanced bright throwing-power, ductility and smoothness. Again, where the disulfonamide is used without the brightener, it produces semi-bright deposits having good semi-bright throwing power, excellent ductility and a good smoothing action.

30 The preferred basic solutions in connection with which the invention is realized are as follows:

#### All sulfate

35 NiSO<sub>4</sub>·7H<sub>2</sub>O ----- 100 to 400 g., preferably 200 to 300 g.  
Boric acid ----- 0 to 60 g., preferably 10 to 40 g.  
Wetting agent (e. g., sodium lauryl sulfate) ----- 0 to 0.5 g., preferably 0.05 to 0.2 g.  
H<sub>2</sub>O to make 1000 cc.

#### All chloride

40 NiCl<sub>2</sub>·6H<sub>2</sub>O ----- 50 to 250 g., preferably 100 to 200 g.  
Boric acid ----- 0 to 60 g., preferably 10 to 40 g.  
Wetting agent (e. g., sodium lauryl sulfate) ----- 0 to 0.5 g., preferably 0.05 to 0.2 g.  
H<sub>2</sub>O to make 1000 cc.

#### Sulfate-chloride (Watts type)

45 NiSO<sub>4</sub>·7H<sub>2</sub>O ----- 100 to 400 g., preferably 200 to 300 g.  
NiCl<sub>2</sub>·6H<sub>2</sub>O ----- 10 to 60 g., preferably 25 to 40 g.  
Boric acid ----- 0 to 50 g., preferably 15 to 40 g.  
Wetting agent (e. g., sodium lauryl sulfate) ----- 0 to 0.5 g., preferably 0.025 to 0.2 g.  
H<sub>2</sub>O to make 1000 cc.

55 To each of the foregoing basic solutions may be added a quantity of the disulfonamide and, if full brightness is desired, a quantity of a brightener and, optionally, a carrier of the aromatic sulfonate or aromatic sulfonamide type.

60 The following specific examples of plating solutions will serve to illustrate the invention, it being understood that the various examples listed above are interchangeable in the following solutions with addition agents of the same class (carrier or auxiliary brightener) and give similar results although some of the compounds of Table I do give very superior results especially in some instances as herein elsewhere indicated.

#### EXAMPLE I (Semi-Bright)

|                                      |          |     |
|--------------------------------------|----------|-----|
| NiSO <sub>4</sub> ·6H <sub>2</sub> O | grams    | 240 |
| NiCl <sub>2</sub> ·6H <sub>2</sub> O | do       | 40  |
| H <sub>3</sub> BO <sub>3</sub>       | do       | 40  |
| Dibenzenesulfonamide                 | do       | 2   |
| pH                                   |          | 3.5 |
| Temperature                          | ° F.     | 140 |
| Cathode current density              | A. S. F. | 40  |
| H <sub>2</sub> O to make one liter.  |          |     |

7  
EXAMPLE II (Semi-Bright)

|                                      |          |     |
|--------------------------------------|----------|-----|
| NiSO <sub>4</sub> .6H <sub>2</sub> O | grams    | 240 |
| NiCl <sub>2</sub> .6H <sub>2</sub> O | do       | 40  |
| H <sub>3</sub> BO <sub>3</sub>       | do       | 40  |
| Dibenzenesulfonamide                 | do       | 6   |
| pH                                   |          | 3.5 |
| Temperature                          | ° F      | 140 |
| Cathode current density              | A. S. F. | 40  |
| H <sub>2</sub> O to make one liter.  |          |     |

## EXAMPLE III (All Chloride-Bright Semi-Bright)

|                                      |          |     |
|--------------------------------------|----------|-----|
| NiCl <sub>2</sub> .6H <sub>2</sub> O | grams    | 300 |
| H <sub>3</sub> BO <sub>3</sub>       | do       | 50  |
| Dibenzenesulfonamide                 | do       | 2   |
| pH                                   |          | 3.5 |
| Temperature                          | ° F      | 140 |
| Cathode current density              | A. S. F. | 40  |
| H <sub>2</sub> O to make one liter.  |          |     |

## EXAMPLE IV (Bright)

|                                      |          |      |
|--------------------------------------|----------|------|
| NiSO <sub>4</sub> .6H <sub>2</sub> O | grams    | 240  |
| NiCl <sub>2</sub> .6H <sub>2</sub> O | do       | 40   |
| H <sub>3</sub> BO <sub>3</sub>       | do       | 40   |
| Dibenzenesulfonamide                 | do       | 0.5  |
| Ethylene cyanohydrin                 | do       | 0.24 |
| pH                                   |          | 3.5  |
| Temperature                          | ° F      | 140  |
| Cathode current density              | A. S. F. | 40   |
| H <sub>2</sub> O to make one liter.  |          |      |

## EXAMPLE V (Bright)

|                                      |          |       |
|--------------------------------------|----------|-------|
| NiSO <sub>4</sub> .6H <sub>2</sub> O | grams    | 240   |
| NiCl <sub>2</sub> .6H <sub>2</sub> O | do       | 40    |
| H <sub>3</sub> BO <sub>3</sub>       | do       | 40    |
| Dibenzenesulfonamide                 | do       | 0.5   |
| Naphthalene disulfonate              | do       | 4     |
| Triaminotriphenyl methane            | do       | 0.005 |
| pH                                   |          | 3.2   |
| Temperature                          | ° F      | 140   |
| Cathode current density              | A. S. F. | 40    |
| H <sub>2</sub> O to make one liter.  |          |       |

## EXAMPLE VI (Bright)

|                                      |          |     |
|--------------------------------------|----------|-----|
| NiSO <sub>4</sub> .6H <sub>2</sub> O | grams    | 240 |
| NiCl <sub>2</sub> .6H <sub>2</sub> O | do       | 40  |
| H <sub>3</sub> BO <sub>3</sub>       | do       | 40  |
| Dibenzenesulfonamide                 | do       | 0.5 |
| Benzaldehyde                         | do       | 0.4 |
| pH                                   |          | 3.5 |
| Temperature                          | ° F      | 140 |
| Cathode current density              | A. S. F. | 40  |
| H <sub>2</sub> O to make one liter.  |          |     |

## EXAMPLE VII (Bright)

|                                                                                 |          |       |
|---------------------------------------------------------------------------------|----------|-------|
| NiSO <sub>4</sub> .6H <sub>2</sub> O                                            | grams    | 240   |
| NiCl <sub>2</sub> .6H <sub>2</sub> O                                            | do       | 40    |
| H <sub>3</sub> BO <sub>3</sub>                                                  | do       | 40    |
| Naphthalene benzene disulfonamide (N-phenyl sulfonyl-2-naphthalene sulfonamide) | grams    | 0.3   |
| Triaminotriphenyl methane                                                       | do       | 0.005 |
| pH                                                                              |          | 3.5   |
| Temperature                                                                     | ° F      | 140   |
| Cathode current density                                                         | A. S. F. | 40    |
| H <sub>2</sub> O to make one liter.                                             |          |       |

## EXAMPLE VIII (Semi-Bright)

|                                                                                                                  |          |     |
|------------------------------------------------------------------------------------------------------------------|----------|-----|
| NiSO <sub>4</sub> .6H <sub>2</sub> O                                                                             | grams    | 240 |
| NiCl <sub>2</sub> .6H <sub>2</sub> O                                                                             | do       | 40  |
| H <sub>3</sub> BO <sub>3</sub>                                                                                   | do       | 40  |
| Cl <sub>2</sub> C <sub>6</sub> H <sub>5</sub> SO <sub>2</sub> NHSO <sub>2</sub> C <sub>6</sub> H <sub>4</sub> Cl | do       | 0.5 |
| pH                                                                                                               |          | 3.5 |
| Temperature                                                                                                      | ° F      | 140 |
| Cathode current density                                                                                          | A. S. F. | 40  |
| H <sub>2</sub> O to make one liter.                                                                              |          |     |

## 8

Having thus described my invention, what I claim is:

1. An acid, nickel electroplating solution comprising a nickel electrolyte of the class consisting of nickel sulfate, nickel chloride and mixtures thereof, together with an addition agent of the formula R—SO<sub>2</sub>NHSO<sub>2</sub>—R', where R is an aromatic radical having not more than ten nuclear carbon atoms and R' is selected from the class consisting of aromatic radicals having not more than ten nuclear carbon atoms, aliphatic radicals having from 1 to 18 carbon atoms, including at least one unsaturated carbon to carbon bond, aryl substituted aliphatic radicals having 7 to 11 carbon atoms, radicals of the formula R''—SO<sub>2</sub>NHSO<sub>2</sub>—R''', radicals of the formula RR''—SO<sub>2</sub>NHSO<sub>2</sub>—R''', radicals of the formula ROR''—SO<sub>2</sub>NHSO<sub>2</sub>—R''' and radicals of the formula RCH<sub>2</sub>R''—SO<sub>2</sub>NHSO<sub>2</sub>—R''', R, R'' and R''' occurring in said last four radicals, indicating aromatic radicals having not more than ten nuclear carbon atoms, said addition agent being present to the extent of from 0.1 to 6 grams per liter.

2. The process of electroplating metallic surfaces by electrolytic deposition from nickel salt solution which comprises passing current to said metallic surface as a cathode through said solution containing as an additive a compound of the formula R—SO<sub>2</sub>NHSO<sub>2</sub>—R', where R is an aromatic radical having not more than ten nuclear carbon atoms and R' is selected from the class consisting of aromatic radicals having not more than ten nuclear carbon atoms, aliphatic radicals having from 1 to 18 carbon atoms including at least one unsaturated carbon to carbon bond, aryl substituted aliphatic radicals having 7 to 11 carbon atoms, radicals of the formula R''—SO<sub>2</sub>NHSO<sub>2</sub>—R''', radicals of the formula RR''—SO<sub>2</sub>NHSO<sub>2</sub>—R''' occurring in said last four radicals indicating aromatic radicals having not more than ten nuclear carbon atoms, said addition agent being present to the extent of from 0.1 to 6 grams per liter.

3. An acid, nickel electroplating solution comprising a nickel electrolyte of the class consisting of nickel sulfate, nickel chloride and mixtures thereof, together with an addition agent having the formula R—SO<sub>2</sub>NHSO<sub>2</sub>—R'

where R and R' are aromatic radicals having not more than ten nuclear carbon atoms, said addition agent being present to the extent of from 0.1 to 6 grams per liter.

4. An acid, nickel electroplating solution comprising a nickel electrolyte of the class consisting of nickel sulfate, nickel chloride and mixtures thereof, together with an addition agent having the formula R—SO<sub>2</sub>NHSO<sub>2</sub>—R'

where R is an aromatic radical having not more than ten nuclear carbon atoms and R' is an aliphatic radical having from 1 to 18 carbon atoms and containing at least one unsaturated carbon to carbon bond, said addition agent being present to the extent of from 0.1 to 6 grams per liter.

5. An acid, nickel electroplating solution comprising a nickel electrolyte of the class consisting of nickel sulfate, nickel chloride and mixtures thereof, together with an addition agent having the formula R—SO<sub>2</sub>NHSO<sub>2</sub>R'—SO<sub>2</sub>NHSO<sub>2</sub>—R''

where R, R' and R'' are aromatic radicals having not more than ten nuclear carbon atoms, said addition agent being present to the extent of from 0.1 to 6 grams per liter.

6. An acid, nickel electroplating solution comprising a nickel electrolyte of the class consisting of nickel sul-

fate, nickel chloride and mixtures thereof, together with an addition agent having the formula



where R, R', R'' and R''' are aromatic radicals having not more than ten nuclear carbon atoms, R' and R'' being connected through nuclear carbon, said addition agent being present to the extent of from 0.1 to 6 grams per liter.

7. An acid, nickel electroplating solution comprising a nickel electrolyte of the class consisting of nickel sulfate, nickel chloride and mixtures thereof, together with an addition agent having the formula



where R is an aromatic radical having not more than ten nuclear carbon atoms and R' is an aryl substituted aliphatic radical having from 7 to 11 carbon atoms, said addition agent being present to the extent of from 0.1 to 6 grams per liter.

8. An acid, nickel electroplating solution comprising a nickel electrolyte of the class consisting of nickel sulfate, nickel chloride and mixtures thereof, together with an addition agent having the formula:



n and n' each indicating an integer from 0 to 3, and the sum of n plus n' not exceeding 3, said addition agent being present to the extent of from 0.1 to 6 grams per liter.

9. An acid, nickel electroplating solution comprising a nickel electrolyte of the class consisting of nickel sulfate, nickel chloride and mixtures thereof, together with an addition agent having the formula:



n and n' each indicating an integer from 0 to 3, and the sum of n plus n' not exceeding 3, said addition agent being present to the extent of from 0.1 to 6 grams per liter.

10. An acid, nickel electroplating solution comprising a nickel electrolyte of the class consisting of nickel sulfate, nickel chloride and mixtures thereof, together with an addition agent having the formula:



n and n' each indicating an integer from 0 to 3, and the sum of n plus n' not exceeding 3, said addition agent being present to the extent of from 0.1 to 6 grams per liter.

11. An acid, nickel electroplating solution comprising a nickel electrolyte of the class consisting of nickel sul-

fate, nickel chloride and mixtures thereof, together with an addition agent having the formula:



n and n' each indicating an integer from 0 to 3, and the sum of n plus n' not exceeding 6, said addition agent being present to the extent of from 0.1 to 6 grams per liter.

10. 12. An acid, nickel electroplating solution comprising a nickel electrolyte of the class consisting of nickel sulfate, nickel chloride and mixtures thereof, together with an addition agent having the formula:



said addition agent being present to the extent of from 0.1 to 6 grams per liter.

13. An acid, nickel electroplating solution comprising a nickel electrolyte of the class consisting of nickel sulfate, nickel chloride and mixtures thereof, together with an addition agent having the formula:



n and n' each indicating an integer from 0 to 1, said addition agent being present to the extent of from 0.1 to 6 grams per liter.

14. The invention as defined in claim 1 wherein said addition agent is  $\text{PhSO}_2\text{NHSO}_2\text{Ph}$ .

15. The invention as defined in claim 1 wherein said addition agent is



16. The invention as defined in claim 1 wherein said addition agent is



17. The process of electroplating metallic surfaces by electrolytic deposition from nickel salt solutions which comprises passing current to said metallic surface as a cathode through said solution containing as an additive



50 said additive being present in said solution to the extent of 0.1 gram per liter.

#### References Cited in the file of this patent

#### UNITED STATES PATENTS

|           |       |               |
|-----------|-------|---------------|
| 2,191,813 | Brown | Feb. 27, 1940 |
| 2,467,580 | Brown | Apr. 19, 1949 |
| 2,644,788 | Shenk | July 7, 1953  |
| 2,644,789 | Shenk | July 7, 1953  |